

July 19, 1938.

H. A. LEWIS ET AL

2,124,201

EXPLOSIVE COMPOSITION AND PROCESS OF PRODUCTION

Filed Sept. 15, 1934



H.A.Lewis INVENTORS

C.A.Woodbury

BY

*Frank J. Glensoske*

ATTORNEY.

## UNITED STATES PATENT OFFICE

2,124,201

EXPLOSIVE COMPOSITION AND PROCESS  
OF PRODUCTION

Harold A. Lewis, Brandywine Summit, and Clifford A. Woodbury, Media, Pa., assignors to E. I. du Pont de Nemours &amp; Company, Wilmington, Del., a corporation of Delaware

Application September 15, 1934, Serial No. 744,100

10 Claims. (Cl. 52—14)

This invention relates to a new and improved explosive composition and to a process for controlling the density thereof, said composition being characterized by relatively high density and a desirable and controllable degree of sensitivity throughout.

Under certain conditions of use, relatively high density is a very desirable property of explosives, since it allows a concentration of explosive strength within a smaller volume of borehole. This is particularly the case in hard rock blasting and in quarrying operations using well drill holes. Where high density is desired, gelatin dynamite has heretofore been the ideal explosive from the point of view of efficiency. From an economical point of view, however, it has been the practice to replace gelatin dynamites, wherever possible, by other, lower cost explosives, particularly those having an ammonium nitrate base. Such ammonia dynamites, unfortunately do not have the desired high density of loading, particularly the economically favorable ones with a low nitroglycerin content. High density ammonium nitrate explosives can, of course, be produced by pressing or casting the charge, but such highly compressed compositions are in general too insensitive for satisfactory detonation with the usual blasting caps.

An object of our invention is an explosive composition of relatively high density and of high bulk strength. A further object is such an explosive characterized by a degree of sensitiveness throughout which is more completely controlled than is usually the case with such high density explosives. A further object is an ammonium nitrate explosive having the properties described herein. A still further object is a process for producing such explosives of controlled density and sensitiveness. Additional objects will be disclosed as the invention is described hereinafter.

We have found that the foregoing objects are accomplished when the explosive composition is produced by using therein a portion of relatively high density pellets of explosive material with a mass of more readily detonatable explosive material, the latter material being in contact with the pellets, and wholly or substantially surrounding them. A principal advantage of this arrangement is that, by using high density pellets the average density of the entire composition is markedly increased while at the same time the sensitiveness of the combination may be controlled to any desired degree.

Our invention is therefore applicable to various types of explosive compositions. It may comprise

a chlorate or perchlorate explosive composition in compressed form such as to give a density higher than that of the remaining composition. Our high density component, however, preferably consists of a compressed explosive in pelleted or granular form, containing ammonium nitrate as the principal ingredient, together with a sufficient amount of sensitizing and oxygen balancing material so that the detonation wave communicated to these pellets by the surrounding explosive composition will be propagated throughout the mass. These pellets may be made solely of ammonium nitrate, but we preferably incorporate with the ammonium nitrate one or more of the carbon compounds to compensate for the excess oxygen produced upon detonation of the ammonium nitrate.

Likewise the surrounding explosive composition may consist of various types of explosives which in themselves have varying degrees of sensitiveness, the principal requirement being that it is more readily detonatable than the pelleted composition used. These surrounding compositions may be more readily detonatable because of their composition or by virtue of lower density. For example when the pellets comprise ammonium nitrate compositions, the surrounding composition may be a gelatin dynamite, a semi-gelatinous dynamite, an ammonium nitrate dynamite which is cap sensitive, or an explosive incapable of detonation by a commercial blasting cap but detonatable by a dynamite primer. Also when the pellets are chlorate explosives, the surrounding explosive is preferably a chlorate composition, in loose form, of lower density, or a lower degree of compression. It will be apparent from the foregoing that innumerable combinations will come within the scope of our invention.

While the most satisfactory procedure in bringing the pellets and the more readily detonatable portions of the explosives into suitable contact with one another will be to enclose the former within the latter material, for the purpose of our invention it is essential only that the pelleted material be contacted by the more readily detonatable material, so that the explosion, when once initiated, is propagated throughout the composition, the more sensitive explosive acting as the carrier of the detonating wave. Such extent of contact may be termed "substantially surrounded" for the purpose of suitable definition.

In preparing an explosive according to this invention, in which the pelleted portion comprises an ammonium nitrate explosive, we find it satis-

factory to use in such portion more than 50% ammonium nitrate and preferably at least 85% of this compound. Various sensitizing materials may be utilized, that are capable of oxidation by ammonium nitrate, such as carbonaceous ingredients, inorganic metallic materials such as powdered aluminum, ferro-silicon or calcium silicide, aromatic nitrocompounds, or even small percentages of explosive compounds such as aliphatic nitric esters, nitroglycerin, ethylene glycol dinitrate, nitrostarch, pentaerythritol tetranitrate and the like. Preferably, however, we employ nitrated aromatic hydrocarbons, for example dinitrotoluene or other nitrotoluene, together with a paraffin hydrocarbon. A satisfactory composition has been found to consist of 92% ammonium nitrate, 4% dinitrotoluene, and 4% paraffin. The amounts of dinitrotoluene and paraffin may be varied, preferably to include dinitrotoluene in amounts up to 20% and paraffin up to amounts of 8%. Increasing the amount of dinitrotoluene gives an increased degree of sensitiveness to the composition, and still permits high densities. Decreasing this and increasing the paraffin content, on the other hand, has the reverse effect. Compressed charges such as these will be too insensitive for detonation by means of a commercial blasting cap but will develop full blasting efficiency when subjected to the detonating action of the surrounding, more sensitive explosive.

The pelleted compositions can be formed by any desired method, as for example by compressing or casting, and, while the density may vary over a wide range, a suitable density may be between 1.4 and 1.5. The size of the pellets can also be varied widely as desired, although for our purpose a satisfactory one may be of cylindrical form with a diameter of about  $\frac{1}{8}$ " and a length of  $\frac{1}{8}$ ".

Another method of forming the pellets is to compress the material to any predetermined density in the form of blocks or cakes, breaking these down, for example by means of cracking rolls, and passing the product over screens to obtain the desired size of pellets or grains.

An ammonium nitrate explosive containing a relatively small amount of nitroglycerin or other aliphatic liquid nitric ester as sensitizing material is suitable for the more readily detonatable portion of the charge. Satisfactory compositions for such use may be more fully illustrated by the following formulae:—

|                                   | 1                | 2                    | 3               | 4                             |
|-----------------------------------|------------------|----------------------|-----------------|-------------------------------|
|                                   | Ammonia dynamite | Ammonia semi-gelatin | Ammonia gelatin | Low sensitiveness composition |
| 60 Nitroglycerin                  | 15.0             | 18.0                 | 35.0            | -----                         |
| Nitrocotton                       |                  | 0.2                  | 1.0             | -----                         |
| Ammonium nitrate                  | 77.0             | 66.0                 | 20.0            | 92.0                          |
| Sodium nitrate                    |                  |                      |                 | -----                         |
| Soda                              |                  | 10.0                 | 33.5            | -----                         |
| Carbonaceous combustible material | 7.5              | 5.3                  | 10.0            | -----                         |
| Chalk                             | 0.5              | 0.5                  | 0.5             | 4.0                           |
| Dinitrotoluene                    |                  |                      |                 | 4.0                           |
| Paraffin                          |                  |                      |                 | 4.0                           |

Examples 1, 2 and 3 above, because of their compositions, are readily detonatable by the commercial blasting caps commonly used, and the composition of Example 4, in loose form, is more readily detonatable than the same composition in pelleted form, and can be detonated by a dynamite primer. The mixing of the two pre-

portions to form the finished composition may be brought about in any desired way.

In the way of further illustrations of our invention the following examples are given of actual mixings having suitable properties and which gave satisfactory performance. Blends containing respectively, 0, 20, and 40% ammonium nitrate pellets surrounded with a low density ammonia dynamite containing 5% nitroglycerin, 87% ammonium nitrate, 7.5% combustible material and 0.5 chalk had the following densities:

| Pellets (percent) | Density |
|-------------------|---------|
| 0                 | 1.03    |
| 20                | 1.10    |
| 40                | 1.16    |

Similarly, a blend containing respectively, 0, 20, and 40% ammonium nitrate pellets surrounded with a low density ammonia dynamite containing 15% nitroglycerin, 77% ammonium nitrate, 7.5% combustibles and 0.5% chalk gave the following densities:

| Pellets (percent) | Density |
|-------------------|---------|
| 0                 | 1.18    |
| 20                | 1.24    |
| 40                | 1.28    |

We may also use liquid nitric esters, such as nitroglycerin or nitroglycol, as the surrounding medium for the pelleted material, such as ammonium nitrate.

It will therefore be seen that our invention has many unique advantages. Ammonium nitrate, for example, is not water-resistant. By our method an explosive is produced wherein the ammonium nitrate can be surrounded by a water-resistant medium, such as gelatin dynamite or liquid nitroglycerin.

As indicated in the foregoing, while we may use pellets of ammonium nitrate only, we have found that our invention may be efficiently practiced by including pellets of ammonium nitrate containing sensitizing materials in order to get rid of the excess oxygen that the ammonium nitrate contains.

Furthermore, the pellets contemplated by our invention may or may not be sufficiently sensitive for detonation by means of a commercial blasting cap.

Our invention therefore in its broadest aspects contemplates an explosive charge which comprises a multiplicity of individual charges of separate explosives, these being substantially surrounded by another explosive which has a higher degree of sensitiveness and which acts as a detonating agent for the individual charges.

The advantages of our invention, as described in the foregoing, will be readily apparent. The surrounding explosive portion is satisfactory for use from the point of view of sensitiveness in that any sensitiveness can be selected, and any other properties, such as varying degrees of water resistance, can be selected as desired. However, many of these types which may be selected are unsuitable and unsatisfactory for blasting in hard rock because of their low density. This latter difficulty is overcome by the pelleted composi-

tion which imparts satisfactorily high density to the entire composition.

Preferably, we use the proportions by means of which maximum density increase is obtained. 5 This maximum density may occur between 30% and 80% of pelleted material. It will be apparent from the foregoing that the explosive properties may be very conveniently controlled by varying the ratio of high density to the surrounding 10 composition.

Heretofore it has been necessary, when high densities are required, to use gelatinous explosives, or high-content nitroglycerin explosives, which compositions are relatively expensive. The present invention for the first time enables compositions 15 containing large amounts of ammonium nitrate and low percentages of nitroglycerin to replace those high density dynamites satisfactorily.

20 For the purpose of more fully illustrating one specific embodiment of our invention, reference may be made to the accompanying drawing in which the single figure shows a container A with a portion cut away to reveal one arrangement 25 of the explosive pellets B substantially surrounded by the more easily detonatable explosive material C. This embodiment of our invention is, however, to be taken as merely illustrative and not as limiting in any way the broad principles of our 30 invention.

While we have described various modifications and embodiments of our invention in detail in the foregoing, it will be apparent therefrom that still further variations may be made in the 35 method of procedure, in the size, shape and density of the less sensitive portion, and in the compositions used, within the scope and spirit of our invention. It is to be understood, therefore that we do not intend to be limited, except 40 as indicated in the following patent claims:

We claim:

1. An explosive composition comprising an explosive matrix capable of sustaining propagation of the explosion upon initiation, and embedded 45 in said matrix, aggregates comprising ammonium nitrate intermingled with an oxygen acceptor and compacted therewith to a density of at least 1.4.

2. An explosive composition comprising a 50 matrix of a nitroglycerin explosive, and embedded in said matrix, aggregates comprising ammonium nitrate intermingled with an oxygen acceptor and compacted therewith to a density of at least 1.4.

55 3. An explosive composition comprising an explosive matrix capable of sustaining propagation of the explosion upon initiation, and embedded in said matrix, aggregates comprising more than

50% ammonium nitrate intermingled with a nitrotoluene and a paraffin hydrocarbon and compacted therewith to a density of at least 1.4.

4. An explosive composition comprising an explosive matrix capable of sustaining propagation 5 of the explosive upon initiation, and embedded in said matrix, aggregates comprising more than 50% ammonium nitrate intermingled with 0.5-10.0% of a nitrotoluene and 0.5-10.0% of a paraffin hydrocarbon and compacted therewith 10 to a density of at least 1.4.

5. An explosive composition comprising a plurality of compact explosive aggregates embedded in an explosive matrix capable of initiation by means of a commercial blasting cap, said aggregates comprising ammonium nitrate intermingled with an oxygen acceptor and compacted therewith to a density of at least 1.4, said aggregates 15 having in themselves a sensitiveness insufficient to insure initiation by means of a commercial blasting cap. 20

6. The explosive composition of claim 5 wherein said oxygen acceptor comprises a mixture of a nitrotoluene and a paraffin hydrocarbon.

7. The explosive charge of claim 5 wherein 25 said explosive matrix capable of initiation by means of a blasting cap comprises a nitroglycerin explosive.

8. The process of producing an explosive composition which comprises intimately mixing ammonium nitrate with an oxygen acceptor and compressing the resulting composition to form a plurality of compact aggregates at the relatively 30 high density of at least 1.4, and embedding said aggregates in an explosive matrix capable of sustaining propagation of the explosion upon initiation. 35

9. The process of producing an explosive composition which comprises intimately mixing ammonium nitrate with an oxygen acceptor and 40 compressing the resulting composition to form a plurality of compact aggregates at the relatively high density of at least 1.4, said aggregates having a sensitiveness insufficient to insure initiation by means of a commercial blasting cap, and embedding said aggregates in an explosive matrix capable of 45 sustaining propagation of the explosion upon initiation.

10. The process of producing an explosive composition which comprises intimately mixing ammonium nitrate with an oxygen acceptor and 50 compressing the resulting composition to form a plurality of compact aggregates at the relatively high density of at least 1.4, and embedding said aggregates in an explosive matrix capable of initiation by means of a commercial blasting cap. 55

HAROLD A. LEWIS.

CLIFFORD A. WOODBURY.